

# UNITED STATES PATENT OFFICE.

VLADIMIR SCHEWELIN, OF MOSCOW, RUSSIA.

## PROCESS OF PRODUCING AN INSULATING MATERIAL.

1,235,061.

Specification of Letters Patent. Patented July 31, 1917.

No Drawing.

Application filed July 9, 1914. Serial No. 849,880.

*To all whom it may concern:*

Be it known that I, VLADIMIR SCHEWELIN, a subject of the Emperor of Russia, and a resident of the city of Moscow, Russia, have 5 invented new and useful Improvements in Processes of Producing an Insulating Material, of which the following is a specification.

This invention relates to an improved 10 process of manufacturing a known insulating filling material for refrigerating cars, passenger cars, acoustic insulation purposes, and the like, which insulating material consists of layers of flax or hemp with interposed sheets of paper, pasteboard, or the 15 like, the layers being thread sewn in different directions.

Hitherto, in refrigerating apparatus, an 20 insulating filling substance known as "lino-felt", has been used, which consists of two layers of water-proof pasteboard, between which is interposed, a thin layer of fine and short flax that contains a considerable quantity of shive.

25 The filling material made in accordance with the present invention is similar in appearance to that above described, but it possesses a higher power of insulation, greater purity, is not so liable to be attacked by mold, 30 and offers greater resistance to shocks and vibrations, to which the filling layers of refrigerating and passenger cars are particularly subjected.

35 In carrying out my invention, the fibrous flax material, and the threads to be used in sewing together the several flax layers of the filling material, are washed in a washing machine at a temperature not below 30 to 40 degrees centigrade, dried by centrifugal force, then lixiviated in a mixture of caustic

soda and calcined soda, and thereupon subjected about three times to a washing operation in hot water, disinfecting and non-odor developing materials, such as borax, perborate, acetate of alumina, and the like, being 45 added during the last washing operation. Finally, the material is subjected to the action of centrifugal force and quickly dried by the addition of formalin vapors.

This treatment results in a pure flax material which is entirely devoid of odor, and is not influenced by moisture or attacked by mold; it yields a large quantity of fiber and possesses superior properties of insulation and resistance against shocks and vibrations. 50 55

The fibrous material produced as described, is formed into a number of layers between which are interposed, sheets of paper, parchment or pasteboard. The composite body thus obtained, is placed between 60 covers of water-proof pasteboard, or textile material, and is connected thereto by means of longitudinal and cross seams.

It is to be understood that my process is not restricted to the use of flax or hemp, 65 as any other fibrous material of similar physical properties may be used instead.

I claim:

A process of treating fiber for use in an insulating filling material which consists in 70 washing the fibrous substance, drying the same, lixiviating it in a mixture of caustic and calcined soda, again washing it in hot water together with disinfecting and non-odor developing substances, and drying it 75 by the addition of formalin vapors.

VLADIMIR SCHEWELIN.

Witnesses:

CHRIST. ERFURT,  
LYDIA RÖLL.

Copies of this patent may be obtained for five cents each, by addressing the "Commissioner of Patents,  
Washington, D. C."